

July 9, 1963

L. B. HALL

3,097,169

SOLID BULLET LUBRICANT

Filed May 27, 1960



LESLIE B. HALL  
INVENTOR.

BY

Richard C. Babcock

ATTORNEY

1

3,097,169

**SOLID BULLET LUBRICANT**

Leslie B. Hall, 817 Grand Ave., Long Beach 4, Calif.  
Filed May 27, 1960, Ser. No. 32,483  
1 Claim. (Cl. 252—23)

The present invention relates generally to the field of lubricants, and more particularly to a lubricant for solid bullets.

A primary object of the present invention is to provide a lubricant of such consistency that it will remain in the solid state in the grooves or cannelures of a bullet missile at normally encountered atmospheric temperatures, but is also capable, when molten, of impregnating the felt filler wads of shotgun shells.

Another object of the invention is to provide a lubricant which, when used on bullets, will cause the gun barrels through which they are fired to acquire a highly polished mirror-like gloss on the interior surface thereof, which gloss not only offers a minimum of frictional resistance to bullet missiles thereafter fired through the barrels, but inhibits the formation of rust in the barrels, as well as the corrosion thereof.

A still further object of the invention is to provide a lubricant that not only provides the operational advantages above mentioned, but one that in addition actually cleans the gun barrels, thus eliminating the necessity of using corrosive lead and nitro solvents thereon.

These and other objects and advantages of the invention will become apparent from the following description of the invention, and the drawing illustrating the same in which:

FIGURE 1 shows a side elevational view of a bullet missile as removed from the mold;

FIGURE 2 shows the bullet missile illustrated in FIGURE 1 after it has been trimmed to correct caliber with its cannelure therein filled with the lubricant of the present invention;

FIGURE 3 is a side elevational view of the bullet missile shown in FIGURE 2, mounted at the correct depth in a shell casing, a portion of which is cut away;

FIGURE 4 is a top plan view of a felt filler wad impregnated with the lubricant; and

FIGURE 5 is a side elevational view of a shotgun shell partially cut away to show the positioning therein of the wad illustrated in FIGURE 4.

In its preferred form the invention consists of grease, beeswax, paraffin, powdered mica, colloidal graphite and oil. All the ingredients, with the exception of the mica and graphite, are liquefied by heating, and all the ingredients are then thoroughly intermixed by agitation.

In preparing the lubricant, the following ingredients are intermixed in the following proportions by weight.

| Ingredients:                      | Parts by weight |
|-----------------------------------|-----------------|
| Grease (type used in water pumps) | 1               |
| Calcium base                      | 1               |
| Soap grease (No. 1 consistency)   | 1               |
| Beeswax                           | 3               |
| Paraffin                          | 4               |
| Powdered mica                     | 3               |
| Graphite (colloidal)              | 1/4             |
| Oil (common hoist)                | 2               |

Intermixing of the above ingredients is effected by heating the same with steam until all thereof except the mica and graphite are in the molten state. Frequent stirring of the ingredients is desirable during the heating operation to assure thorough intermixing thereof. The heating should be continued only sufficiently long for thorough intermixing of the ingredients to take place, and to assure that no lumps or agglomerates remain in the finished lubricant.

2

The grease, of a type used on water pumps, is anhydrous, has a calcium soap content of approximately 7%, excess alkali not over 0.15%, excess free acid not over 0.15%, and enough mineral oil to give it an ASTM No. 1 consistency (ASTM—American Society for Testing Materials). No. 1 consistency approximates that of a heavy salve.

The calcium base soap grease is anhydrous, has a calcium base soap content of 5% to 7%, excess free acid not over 0.15%, excess alkali not over 0.15%, lead oxide 3%, and enough mineral oil to give an ASTM No. 1 consistency.

The proportions of the materials comprising the grease and soap above mentioned are by weight.

15 The beeswax and paraffin preferably have a melting point of 160°—165° F.

The oil, designated as Common Hoist, has an API gravity of 23 (API—American Petroleum Institute); Saybolt viscosity of 200 at 100° F.; flash point of 360° F.; 20 fire point of 450° F.; pour point of 20° F.; and a color of ASTM Union No. 2 (Pale Amber).

In the lubricant compounded as above described, the grease and calcium base soap assist in holding the mica and graphite in suspension and as carrier therefor. The beeswax and paraffin serve as lubricative binders. The oil acts as a thinner, and when varied, permits the hardness of the invention to be controlled.

The mica in the present invention serves as a lubricant, even at the hottest temperatures to which the inside surface of a gun barrel will be subjected, and in addition serves to fill the pores of the metal defining the gun barrel. The colloidal graphite and mica in cooperation act as a lubricant when deposited on the interior surface of a gun barrel. Both the mica and graphite are preferably in a finely divided state to assure even distribution thereof through the grease, soap, beeswax, paraffin and oil during the time they are being heated and subjected to agitation.

30 In use, the lubricant is preferably carried as an integral part of the bullet or shotgun shell as shown in the drawing.

In FIGURE 1 a bullet missile A is shown that has a heel or base 1, lubrication groove or cannelure 2, crimp groove 3, and nose or point 4. FIGURE 2 illustrates a bullet missile A after it has been trimmed to correct caliber, with the groove 2 filled with the lubricant B. The lubricant B may be placed in the groove 2 by use of a conventional bullet lubricator and sizer. Another method is to place the bullet missile A upright in a shallow, flat-bottomed receptacle (not shown) which holds the melted lubricant B. The lubricant B must be of sufficient depth in the receptacle to enter groove 2 but not the crimp groove 3. After the lubricant is allowed to solidify in the receptacle, the bullet missile is removed therefrom, and the excess hardened lubricant in groove 2 trimmed therefrom. Bullet missile A is then seated in shell case 6 above the powder charge, with the upper portion of the case being crimped or swaged into the groove 3.

60 The lubricant is preferably used in shotgun shells by soaking a felt filler wad 8, as shown in FIGURE 4, in the material when it is heated and in the molten state. The length of time the wad 8 is allowed to soak in the liquid lubricant determines the completeness of the impregnation thereof. After wad 8 is impregnated with the lubricant it is placed in a paper shotgun shell case 13 that has a metallic base 9. The impregnated wad 8 is situated above powder charge wad 10 and felt washer 11, but below the shot charge 12. When the lubricant is disposed in the groove 2 or impregnates a wad 8 inside a shell casing 13 it is sealed from contact with the ambient atmosphere, and is accordingly prevented from gathering

dust, dirt and other foreign material that would be harmful to the interior surface of a gun barrel.

The use of the invention has been previously described in detail and need not be repeated. From experience in using the invention it has been found to withstand both high and low temperatures without the ingredients tending to separate, or the lubricant losing oil. Also, the lubricant has the desirable property that it will not smudge the hands.

When used with bullets, the lubricant cleans the gun barrels through which such bullets are fired of lead particles and foreign materials left from previous firings, and also lubricates the bore surfaces of the barrels and imparts a mirror-like gloss thereto that lasts indefinitely. In addition, the lubricant remains intact with the bullet missile, as has been determined by the examination of recovered bullets.

Although the invention herein shown and described is fully capable of achieving the objects and providing the advantages hereinbefore mentioned, it is to be understood that it is merely illustrative of the presently preferred embodiment thereof and that I do not mean to be limited to the details thereof, other than as defined in the appended claim.

I claim:

A lubricant for use in cleansing a small arms barrel when a bullet missile is fired therethrough and also im-

parts a mirror-like gloss to the interior surface of said barrel, said lubricant being capable of filling a circumferentially extending groove in said bullet missile, which lubricant is of sufficiently heavy consistency to permit a major portion of said lubricant to remain in said groove after said missile is fired through said small arms barrel, said lubricant comprising the following ingredients in parts by weight:

|                          | Parts |
|--------------------------|-------|
| Calcium base soap grease | 2     |
| Beeswax                  | 3     |
| Paraffin                 | 4     |
| Finely powdered mica     | 3     |
| Colloidal graphite       | 1/4   |
| Common hoist oil         | 2     |

References Cited in the file of this patent

UNITED STATES PATENTS

|           |           |               |
|-----------|-----------|---------------|
| 681,091   | Adamson   | Aug. 20, 1901 |
| 1,231,227 | Williams  | June 26, 1917 |
| 2,047,897 | Sykes     | July 14, 1936 |
| 2,332,196 | Bjorksten | Oct. 19, 1943 |
| 2,346,124 | Dew       | Apr. 4, 1944  |
| 2,356,367 | Wright    | Aug. 22, 1944 |

FOREIGN PATENTS

|        |               |               |
|--------|---------------|---------------|
| 11,949 | Great Britain | Apr. 20, 1895 |
|--------|---------------|---------------|